

Feb. 6, 1968

R. W. WOODRUFF ET AL

3,367,292

ELECTRIC FURNACE ROOF CONSTRUCTION

Filed Feb. 9, 1966



Fig. 1



Fig. 2

INVENTOR.  
ROGER W. WOODRUFF &  
BEN DAVIES  
BY  
*William C. Nealon*  
ATTORNEY

# United States Patent Office

3,367,292

Patented Feb. 6, 1968

1

3,367,292

ELECTRIC FURNACE ROOF CONSTRUCTION  
Roger W. Woodruff, Bethel Park, and Ben Davies, Pittsburgh, Pa., assignors to Dresser Industries, Inc., Dallas, Tex., a corporation of Delaware

Filed Feb. 9, 1966, Ser. No. 526,091

5 Claims. (Cl. 110—99)

## ABSTRACT OF THE DISCLOSURE

A basic electric furnace roof or a like dish-shaped dome-type furnace roof substantially entirely made of direct-bonded brick having a porosity over 20%, permeability of less than 1.5 units as hereinafter defined, a modulus of rupture at 2300° F. substantially twice that at room temperature and a density of not more than 175 p.c.f.

This invention relates to fabrication of chemically basic electric furnace roofs.

A good treatise on the subject of electric furnaces, the construction of roofs therefor, and the like, is "Electric Furnace Steelmaking, volume 1, Design, Operation, and Practice," published by Interscience Publishers, a division of John Wiley & Sons, Inc., in 1962. It is a product of the "Physical Chemistry of Steelmaking Committee" of The American Institute of Mining, Metallurgical, and Petroleum Engineers. The reader is directed thereto for a discussion of known prior art and, in particular, the section entitled "Roof Construction," beginning on page 163. As this work points out, silica brick and, to a lesser extent, certain types of fire brick and high alumina brick have been the conventional refractories for the roofs of electric steelmaking furnaces. However, with increasingly severe and extended furnace campaigns becoming conventional, such brick are proving of insufficient refractoriness. Basic brick would seem to provide the logical substitute, but usage thereof has been considered replete with difficulties. First, the considerably increased density as one moves from silica (about 120 p.c.f.) to basic (180+ p.c.f.) brick so increases the total weight of a given roof that much existing roof lifting and moving equipment is insufficient.

Thus, it is an object of this invention to provide for basic electric furnace roof construction more readily adaptable to existing electric furnace shops.

Briefly, according to one aspect of this invention, there is provided an electric furnace roof construction of chemically basic fired refractory brick, which is relatively lightweight, but which has the necessary elevated temperature strength for such a roof.

Other details and further features and advantages of this invention will become more readily apparent to those skilled in the art from a study of the following description together with reference to the attached schematic drawing of an electric furnace. In these drawings:

FIG. 1 is a top view of a furnace roof according to the invention; and

FIG. 2 is a side sectional view along the line A—A of the roof of FIG. 1.

Before describing the drawings in detail, it should be understood they are but exemplary of preferred practice according to the concepts of this invention, and are provided for purposes of explanation and not by way of limitation. The true measure of the spirit and scope of the invention is as defined in the hereinafter appended claims.

In FIGS. 1 and 2, there is shown a plurality of concentric rings arranged circumferentially within a circular roof band 20 to form a downwardly-opening dome-type dish-shaped roof. Each of these rings 21 is comprised of a plurality of burned, low-density, magnesia-chrome ore refractory brick as hereinafter defined. The first eleven

2

rings are entirely of brick. The remaining seven are incomplete, but substantially fill the space between the equi-spaced tubular electrode ports 22, 23, and 24. The remainder of the central area between the incomplete rings and the electrode ports is fabricated of a ramming mix 25. In fabrication of the roof, a dome-shaped wooden form or the like is placed on the floor or a comparable supporting surface and the concentric rings are built up, the electrode ports constructed, and the ramming mix likewise installed.

The shapes of the respective brick of each ring are dictated by conventional practice; for example, as shown on p. 507 of the book Modern Refractory Practice, 4th edition, published by the Harbison-Walker Refractories Company, in 1961.

When it was first determined that conventional basic refractory brick could not be used successfully in a dome-shaped electric furnace roof of the type allowing for free rise and fall without substantial distortion, and without special lifting equipment, it was suggested that means of

lightening the overall weight of the roof would be a possible solution. To this end, batches of the type used to make brick of the type disclosed and claimed in U.S. Patent No. 3,180,744 were studied. The first thought was conventional burnout materials would be the best solution to provide lower density brick. The aim was to provide a brick having a density of less than about 150 p.c.f. but, in any event, consistently less than about 180 p.c.f. To this end, a plurality of batches were fabricated using as burnout material coarse coconut shell, ivory nut shell, and walnut shell.

All of the mixes tested had approximately equal size gradation, the only difference from batch to batch being the type of burnout material used. An exemplary batch would have about 10% of a —4+28 mesh burnout material. The batch using the ivory nut shells had about 12% of that material, but also in the same —4+28 mesh size range. The remainder of the batch was suitably size-graded to make an overall satisfactory brickmaking size-graded batch. The overall oxide analysis of the batch was about 60-70% MgO, about 14-20% Cr<sub>2</sub>O<sub>3</sub>, about 4-10% Al<sub>2</sub>O<sub>3</sub>, less than about 3% SiO<sub>2</sub>, about 5-10% FeO, and up to about 3% CaO.

All of the brick batches were tempered with about 3.6% of a 50:50 lignin:water tempering agent, formed into brick on a conventional brick press, and fired at a temperature of about 3050° F.

The mixes were all so designed as to provide a brick of about 150 p.c.f. or less when burned. The mix containing the ivory nut shells was badly disrupted when ejected from the mold box. The mixes containing coconut or walnut shells showed slight pressure cracking and sponginess at the press, and were disrupted when burning. It appeared the natural elasticity of such burnout materials prevented their proper usage in making burned basic brick, particularly direct-bonded basic brick of the type disclosed and claimed in the U.S. patent referred to above.

It was thought that coating the shells with refractory fines and using some of the tempering agent as a glue therefor would make the shells less resilient. Indeed, the coated shells allowed brick to be pressed satisfactorily. However, their high-temperature strength (i.e., modulus of rupture at 2300° F.) averaged about only 430 p.s.i., and the high permeability of 3.9 (allowing undesirable penetration by corrosive furnace fumes) made them far from satisfactory. For this invention, the brick should have an elevated temperature strength at least about twice that at room temperature and a permeability (as herein-after defined) of no more than about 1.5.

Faced with the apparent total failure of conventional techniques for making lightweight brick, other means had to be found to obtain the desired low porosity but also obtain satisfactory elevated temperature strength. Thus,

in additional studies it was decided that the batch ingredients themselves should be so manufactured as to inherently have a high porosity (i.e., be lightweight) and yet not lead to undesirable permeability. The following table illustrates the results of the additional testing.

units. In the practice reported herein, the permeability value represents the volume of dry air, measured at room temperature and atmospheric pressure, which will flow through a one-inch cube of the test material in one second under a pressure differential of one p.s.i. The unit is

TABLE I

|                                                                                                             | A                                          | B                   | C                                   | D                                  | E      |
|-------------------------------------------------------------------------------------------------------------|--------------------------------------------|---------------------|-------------------------------------|------------------------------------|--------|
|                                                                                                             | Power Pressed at 8,000 p.s.i.              |                     | Impact Pressed 10 Seconds 4 Hammers |                                    |        |
| Standard <sup>1</sup>                                                                                       | Standard <sup>1</sup> with Light Magnesite | All Light Magnesite | Light Magnesite With Special Fines  | Light Magnesite With Special Fines |        |
| Mix (percent):                                                                                              |                                            |                     |                                     |                                    |        |
| Magnesite, 4/10                                                                                             | 30                                         |                     |                                     |                                    |        |
| Magnesite, 10/28                                                                                            | 10                                         |                     |                                     |                                    |        |
| Magnesite, Ball Mill Fine (55-60% -325 mesh)                                                                | 30                                         | 33.1                | 44                                  |                                    |        |
| Light Magnesite, 4/10                                                                                       |                                            | 25.7                | 26                                  | 26                                 | 30     |
| Light Magnesite, 10/28                                                                                      |                                            | 8.6                 | 30                                  | 30                                 | 35     |
| Philippine Chrome Ore Concentrates, 6/28                                                                    | 6                                          | 6.6                 |                                     |                                    |        |
| Philippine Chrome Ore Concentrates, -28                                                                     | 24                                         | 26.3                |                                     |                                    |        |
| Grain of Type Disclosed in U.S. Patent No. 3,116,156, Ball Mill Finer (55-60% -325 Mesh)                    |                                            |                     |                                     | 44                                 |        |
| Grain of Type Disclosed in U.S. Patent No. 3,116,156, 3 Microns (Fisher Subsieve Analyzer Average Diameter) |                                            |                     |                                     |                                    | 35     |
| Burn, Temperature, ° F. (10-Hour Hold)                                                                      | 3,050                                      | 3,050               | 3,050                               | 3,050                              | 3,050  |
| Bulk Density, p.c.l. (A.v. 4)                                                                               | 185                                        | 174                 | 153                                 | 172                                | 172    |
| Modulus of Rupture, p.s.i.:                                                                                 |                                            |                     |                                     |                                    |        |
| At Room Temperature                                                                                         | 500                                        | 430                 | 1,840                               | 550                                | 1,020  |
| At 2,300° F. (hold time 5 hours)                                                                            | 950                                        | 910                 | 140                                 | >1,090                             | >1,180 |
| Apparent Porosity, percent                                                                                  | 18.4                                       | 23.5                | 30.4                                | 30.2                               | 25.6   |
| Permeability <sup>2</sup>                                                                                   | 1.4                                        | 1.3                 | 0.47                                | 0.46                               | 1.4    |

<sup>1</sup> According to United States Patent No. 3,180,744.

<sup>2</sup> Breaking capacity of equipment exceeded at this point.

<sup>3</sup> As hereinafter defined.

The testing provided rather surprising results. Superior brick required both careful control of constituents as well as manufacturing procedure. Mix A (according to U.S. Patent No. 3,180,744), as compared to Mix B, was substantially identical except that "light" magnesite was used, and showed considerably lesser density, but equivalent (within experimental error) elevated temperature strength. Brick entirely of the light magnesite (Mix C) were totally unsatisfactory at elevated temperatures. The light magnesite mixed with fused grain (of the type disclosed in U.S. Patent No. 3,116,156) and manufactured into brick (according to teachings of Patent No. 3,199,994) provided even lower density brick having elevated temperature strength which exceeded the breaking capacity of the equipment being used. Mix D is the preferred embodiment of the invention having as it does the lowest permeability with excellent high-temperature strength. Another very desirable characteristic of the brick illustrated by the data is that, despite very high porosity or void area, the permeability (a measure of interconnected void or pore area) is very low. This is, in large part, due to the use of lightweight magnesite grain in which contained pore space is substantially discontinuous. Preferably, the porosity is over 30% and the permeability less than about 0.5%. It is satisfactory that the porosity be above about 20% and the permeability less than about 1.5%.

It is preferred the lightweight, low-density magnesite constitute substantially the coarser -4+28 mesh fraction of the brickmaking batch to assure the maximum amount of contained encapsulated or disconnected pore space therewithin is not broken by crushing too fine in making a sized batch.

From the foregoing tests, permeability was determined substantially as described in the article by G. R. Eusner and J. T. Shapland in "Permeability Of Blast-Furnace Refractories," Journal of the American Ceramic Society, vol. 42, No. 10, pp. 459-464, 1959. In the practice of this invention, the permeability may be expressed in various

stated as cu. in./sec./sq. in. of area/in. thickness/p.s.i. pressure. The following formula is used:

Permeability =

$$40 \frac{\text{flow rate (cc./min.)} \times \text{thickness (in.)} \times 0.00526}{\text{area (in.}^2\text{)} \times \text{pressure (cm. of Hg)}}$$

Thus, essentially, the present invention is based upon fabricating the major portion of a roof of an electric furnace with burned direct-bonded basic refractory shapes having low density but excellent high-temperature strength. This is, in large part, predicated upon using a magnesite having an inherent density of no more than about 2.70. The magnesite must be such that the permeability of the resulting shape is less than about 1.5 permeability units, as above defined. The magnesite and chrome spinel constituents of the burned shapes must be characterized by substantial direct-bonding substantially without intervening silicate filming. The modulus of rupture of the shapes at 2300° F. should be at least about twice that at room temperature. Of course, to properly make such brick the total SiO<sub>2</sub> content of the batch should be maintained at less than about 2%.

The chrome ore used in the tests reported had the following typical chemical analysis:

|                                                  | Percent |
|--------------------------------------------------|---------|
| Silica, (SiO <sub>2</sub> )                      | 2.4     |
| Alumina, (Al <sub>2</sub> O <sub>3</sub> )       | 33.4    |
| Iron Oxide, (FeO)                                | 11.2    |
| Chromic Oxide, (Cr <sub>2</sub> O <sub>3</sub> ) | 35.0    |
| Lime, (CaO)                                      | 0.3     |
| Magnesia, (MgO)                                  | 17.1    |

All magnesite (both dense and lightweight) had the following typical analysis:

|                                               |      |
|-----------------------------------------------|------|
| 70 Silica, (SiO <sub>2</sub> )                | 0.7  |
| Alumina, (Al <sub>2</sub> O <sub>3</sub> )    | 0.3  |
| Iron Oxide, (Fe <sub>2</sub> O <sub>3</sub> ) | 0.3  |
| Lime, (CaO)                                   | 0.9  |
| Magnesia, (MgO)                               | 97.5 |
| 75 Loss on Ignition                           | 0.1  |

In the foregoing discussion, all parts and percentages are by weight, analyses are on an oxide basis, and sizing refers to the Tyler series—unless specifically stated to the contrary.

Having thus described the invention in detail and with sufficient particularity as to enable those skilled in the art to practice it, what is desired to have protected by Letters Patent is set forth in the following claims:

We claim:

1. In an electric furnace roof or the like having a downwardly-opening dish-shaped dome-type roof, said roof being fabricated of a plurality of ceramically bonded basic refractory shapes contained in adjacent concentric rings within a roof band, substantially all of the brick in said roof being direct-bonded brick having a porosity over about 20% but a permeability of less than about 1.5 units as determined by the formula:

Permeability =

$$\frac{\text{flow rate (cc./min.)} \times \text{thickness (in.)} \times 0.00526}{\text{area (in.}^2\text{)} \times \text{pressure (cm. of Hg)}}$$

and a modulus of rupture at 2300° F. substantially twice that at room temperature, the density of each of said plu-

rality of brick in said roof being no more than about 175 p.c.f.

2. The electric furnace roof construction of claim 1 in which the density of said brick is less than about 150 p.c.f.

3. The electric furnace roof construction of claim 1 in which the porosity of said brick is above about 30% and the permeability below about 0.5.

4. The electric furnace roof construction of claim 1 in which said brick are direct-bonded brick made from a size-graded batch of dead-burned low-density lightweight magnesite and low-silica chrome ore.

5. The electric furnace roof construction of claim 4 in which the lightweight magnesite forms substantially all the coarser —4+28 mesh fraction of the batch.

#### References Cited

#### UNITED STATES PATENTS

|           |         |               |       |        |
|-----------|---------|---------------|-------|--------|
| 2,814,476 | 11/1957 | Leitner       | ----- | 263—46 |
| 3,180,744 | 4/1965  | Davies et al. | ----- | 106—59 |
| 3,194,672 | 7/1965  | Davies et al. | ----- | 106—59 |
| 3,309,175 | 3/1967  | Berg et al.   | ----- | 106—58 |

FREDERICK L. MATTESON, JR., *Primary Examiner.*

J. J. CAMBY, *Assistant Examiner.*